# EUROPEAN PATENT SPECIFICATION

(11) **EP 1 345 780 B1**
(45) Date of publication and mention of the grant of the patent: **23.11.2005**
(21) Application number: 01995084.9
(22) Date of filing: 27.12.2001
(51) Int. Cl.: B41M 5/00

(54) **INK JET RECORDING MEDIUM**
TINTENSTRAHLAUFZEICHNUNGSMEDIUM
SUPPORT D'ENREGISTREMENT DE JETS D'ENCRE

(30) Priority: 28.12.2000 EP 00204778
(43) Date of publication of application: 24.09.2003
(73) Proprietor: Fuji Photo Film B.V., 5047 TK Tilburg (NL)
(72) Inventor: VAN DER VELDEN-SCHUERMANS, Bernadette C.A.M., NL-5071 TN Udenhout (NL); DE VRIES, Ieke, NL-5171 WV Kaatsheuvel (NL)
(74) Representative: Prins, Adrianus Willem
(86) International application number: PCT/NL2001/000944
(87) International publication number: WO 2002/053391

(56) References cited:
- WO-A-97/22467
- US-A- 5 605 750
- US-A- 6 020 058
- US-A- 6 025 068

## Description

### Field of invention

The present invention relates generally to an ink jet recording medium, preferably of photographic quality, that has excellent ink absorption speed, good wettability characteristics and a good image printing quality.

### Background of the invention

There are in general two approaches for producing ink jet recording media with photographic quality. Both approaches have unresolved deficiencies and problems.

The conventional approach, the so called "non-microporous film type" ink jet media, is proposed in several patent publications such as DE-A 4322178, EP-A 0806299, JP 2276670, and JP 5024336.

For this type of ink jet recording medium, at least one ink receptive layer is coated on a support such as a paper or a transparent film. The ink receptive layer typically contains various proportions of water soluble binders and fillers. The proportions of these components affect the properties of the coatings e.g. ink absorption properties and the gloss quality appearance of the ink jet media.

One of the important properties of an ink jet receptive coating formulation is the liquid absorptivity. The majority, if not all, of the ink solvent has to be absorbed by the coating layer itself. Only when paper or cloth or cellulose is used as a support, some part of the solvent may be absorbed by the support. It is thus obvious that both the binder and the filler should have a significant ability to absorb the ink solvent.

Another important property for an ink jet recording medium having photographic quality, is its glossiness. It has been a research theme for more than 10 years to find a good balance between a high ink solvent absorptivity and at the same time a high gloss value for an ink jet media.

In WO-A 0/02734 it has been described that the gloss and the permeability properties of the ink receptive coating depend very much on the concentration of the filler volume. Relatively glossy coatings can be achieved when the filler volume is small. This can be realised by choosing relatively small filler particles compared to the coating thickness. However, unless the binder is very hygroscopic, such a coating will be relatively impermeable to ink-solvent. This will result in a long drying time for the ink-solvent. And in some cases, it will lead to an unacceptable smudge problem.

In order to increase the ink-solvent absorbtivity, it is suggested among others in EP-A 0634287, JP 08282088, JP 08/290654, and JP 2000-108501, to coat multiple layers on the support. The first coating layer formed directly on the surface of the support is designed to have a high solvent absorbtivity. The ink receptive layer that is coated as a second layer on top of the first layer, is responsible for a good gloss and colour density. In this design, there are more variables that can be utilised for adjusting the balance between the gloss and ink-solvent absorptivity properties, e.g. the ratio of binder and filler in the ink-receptive layer which in general is lower than that in the layer below; different filler particles and a different filler size for both layers.

Although a significant improvement is seen in the absorbtivity and the gloss appearance, this concept has a major disadvantage in the manufacturing process thereof. The process for manufacturing a multiple coating of filler and binder mixtures on a support is relatively slow. It is believed that the combination of an increase in the coating load and the process to coat the multiple layers containing a large amount of binder and filler particles, have significantly caused the slow manufacturing process.

Recently, a lot of investigations has been directed to the field of ink jet recording media, wherein a hygroscopic microporous membrane is involved. This so called "microporous film type" is superior to the non-microporous type especially due to its high absorption speed for the ink-solvent. By this method the drying time for the ink solvent decreases significantly. US-A 4861644, US-A 5605750, WO-A 9907558 and EP-A 0995611 provide some examples of the methods.

In this microporous type, the microporous film has the primary function to absorb the ink solvent. The typical microporous film suitable for this purpose is described among others in US-A 4833172 and commercially available under the name TESLIN®. The major part of the microporous film comprises precipitated silica particles, which is suitable for absorbing the ink solvent. The hydrophilic microporous films, which are commonly used for filtration purposes are also suitable to be used for the ink solvent absorbing layer.

In US-A-5 605 750 it is suggested to apply an ink receiving layer on top of the microporous membrane in order to increase the color density, glossiness, etc. The coating solution applied in this publication remains on the surface of the microporous film and does not penetrate into the pores of the microporous film.

US-A-6 020 058 describes an ink material wherein on top of the microporous film, a coating solution is coated. This coated solution will stay on the surface in order to enhance the printed image quality with high color fidelity (dry thickness of this layer is around 20 µm). The coating will thus not penetrate into the pores of the microporous film, since it is not meant as an impregnating agent.

One of the disadvantages of these known microporous membranes are their price, which is relatively high. Besides that, the commercially available film has a minimum thickness of 150 µm, which is too thick to be readily laminated onto a base paper support. Hence, it would be necessary to adjust the thickness of the regular photographic base paper support or adjust the process conditions as such that we still be able to produce the photographic ink jet media according to the determined quality standard. Either way, the above mentioned adjustments to existing lamination processes is undesired and economically not favourable.

There are a lot of other microporous films with a comparable void volume which are significantly thinner (thickness less than 150 µm) and cheaper than the said hydrophilic microporous film. In WO-A 9619346, BE-A 1012087, EP-A 0283200 and US-A 4350655 some examples thereof have been described. These microporous films are usually applied in the products that have a limited use and for disposable goods. Examples of such products include medically related products such as surgical drapes and gowns, disposable personal care absorbent products such as diapers and sanitary napkins, protective clothing, sport wears and the like.

The pore structure of said films is permeable for gas, but these films are typically water repellent. It is believed that the water repellent property of these films is caused by the polyolefin resin content of the films which is hydrophobic and the manufacturing method which involving treatment of the filler particles with fatty acids salts, silicone oils or with silanes. The filler particles, which are usually calcium carbonate that is white and low in price, need to be treated in order to make the filler hydrophobic and to obtain a polymer loading amount which is preferably higher than 65 wt%.

There remains a need for having a film that is suitable to be used as an ink solvent absorbing layer for the ink jet media, which properties are a combination of both said microporous films, i.e. a film that is thin enough, has enough void volume, has high ability to absorb the ink solvent and is cheap.

Particularly, there remains a need to have coating solutions that can be applied to various microporous films, which have a thickness of less than 150 µm and which are low in price, in order to maximise its absorption capacity towards an ink-jet ink solvent.

### Summary of the invention

The object of the present invention is to provide an ink jet recording medium comprising a microporous film, said recording medium having advantageous properties in relation to ink absorption speed, wettability characteristics and a image printing quality, more in particular being suited to produce images of photographic quality.

Accordingly the present invention provides an ink jet recording media comprising:
(i) a support, and
(ii) a microporous film adhered to said support, said microporous film being an oriented polyolefin film comprising fillers and having interconnecting channels between the pores, with a void volume between 30 to 90 volume percent of the total microporous film, said microporous film has been impregnated with an aqueous solution comprising at least a water-soluble polymer and surfactant,
(iii) at least one ink receiving layer coated on said impregnated microporous film
(iv) optionally, a protective layer on top of the ink receiving layer.

### Brief description of the drawing

Figure 1 is a cross sectional view of one of the embodiments of the invention.
Figure 2 is another cross-sectional view of the embodiments of the inventions.
Figure 3 is a schematic representation of a plot of surface tension versus the logarithmic value of the surfactant concentration in a water-soluble polymers.

### Detailed description

Figure 1 illustrates one of the embodiments of the invention. Ink jet recording medium 10 comprises of a pre-treated microporous film 11. The microporous film is laminated to a support 14 by means of an adhesive layer 13. Therefore coating and laminating techniques can be applied which are known to those skilled in the art. Non limiting example of such a process is coating the adhesive layer 14 on the support by using a bar coating, gravure coating, roll coating, curtain coating, spray coating, extrusion coating or the like and adhere said microporous film 11 thereon. Thereafter, the aqueous pre-treatment solution is coated on the microporous film prior to coating the ink receiving layer 12. It is still within the spirit of this invention to apply both the pre-treatment aqueous solution and the ink receiving layer 12 at the same time by using one of the multi layers coating methods known to those skilled in the art. It is also in the spirit of the invention to pre-treat the microporous film with said aqueous solution prior to laminate said film on the support.

The microporous layer 11 can be of any porous films produced by the processes involving mixing of thermoplastic polymer with at least one filler, extruding the mixture at an elevated temperature to form a film, optionally pre-stretching the film, cooling the pre-stretched film to solidified the film and stretching the solidified film to form a microporous film. The thickness of the microporous film should be less than 150 µm, preferably between 15 and 150 µm, more preferably between 35 and 100 µm.

Minor amounts, usually less than 15 percent by weight, of other materials may optionally be present in the microporous film. Examples of such materials include matting agents such as titanium dioxide; optical brightener; surfactants; pH controllers, antioxidants, ultraviolet light absorbers, dyes, antistatic agent and the like.

The said microporous film is permeable to gas and is water repellent. Due to its water-repellent properties, it does not have enough absorption speed towards water. Hence, we need to pre-treat said microporous film by a hydrophilic coating solution.

Surprisingly, it has been found that the absorption speed of the microporous film can be increased significantly by applying a coating solution comprising a water-soluble polymer and the appropriate surfactant at a certain concentration.

Without being bound with it, it is believed that pre-treatment of the microporous film with an aqueous solution comprising only a water-soluble polymer will result in a thin film formation on the microporous film. Consequently, a water drop applied on the pre-treated microporous film will not be absorbed into the pores. On the other hand, a coating solution comprising surfactant only will penetrate into the pores and the surfactant molecules will mainly remain in the voids after drying. As consequence, the surface of the microporous film will stay hydrophobic. Pre-treatment of the microporous film by a coating solution containing water-soluble polymer and surfactant thus results in impregnation of said film.

The suitable concentration of the surfactant depends on the amount and kind of the water-soluble polymers. In order to indicate the suitable concentration meant in this invention, we firstly define the terminology critical aggregation concentration (CAC), critical micelle concentration (CMC) and the meaning of those concentration region in a water-soluble polymer / surfactant mixture.

Figure 3 shows a schematic representation of a plot of surface tension versus the logarithmic value of the surfactant concentration, illustrating the position of the transition points. The labelling of these two transition points, T1 and T2, was introduced by M.N. Jones, in "Journals of Colloid and Interfacial Science" number 23 (1967), page 36, in his studies of sodium dodecyl sulphate (SDS) and poly-ethylene-oxide. This is in contrast with aqueous surfactant solution where only one break point at the critical micellization concentration (CMC) is observed. In the article titled Anionic Surfactants; Physical chemistry of surfactant action, which is published in the Surfactant Science Series volume 11, page 109 until 141, edited by E.H. Lucassen-Reynders, it is described that the similar transition points, T1 and T2, are observed for the interaction between SDS and poly-vinyl-pyrrolidone. In the article of D. Muller et al. published in "The Imaging Science Journal", volume 45 (1997) pages 229-235, he shows similar transition points, T1 and T2, in his study on the interaction of gelatin and sodium dodecyl benzene sulphonate.

According to I.P. Purcell et al., in "Colloids and Surfaces"; A: Physicochemical and Engineering Aspects 94 (1995) pages 125-130, the three different regions in figure 3 are generally explained in terms of a polymersurfactant interaction. Initially, at low surfactant concentrations it is thought that single surfactant ions may be binding to the polymer. On increasing the surfactant concentration the first transition point T1 is reached. This point represents the onset of formation of polymer/surfactant complexes. These complexes are believed to consist of surfactant molecules clustered in sub-units which are themselves absorbed on the polymer. On further addition of the surfactant to the solution more of these polymer-bound micelles are formed until the polymer is saturated at T2. At this point the formation of regular surfactant micelles in the solution commences and the behaviour exhibited is then the same as that of pure surfactant solution.

There are various suitable methods for determining the transition points T1 and T2 mentioned above. Besides the surface tension measurement, one can apply the conductivity measurement, the viscosity measurement, the turbidity measurement and dye absorption spectra measurement.

For the purpose of this invention, "critical aggregation concentration (CAC)" means the first transition point T1, where the complex formation of water-soluble polymer and surfactant aggregates starts.

For the purpose of this invention, "critical micelle concentration (CMC)" means the second transition points T2, where the formation of regular surfactant micelles in the solution starts. The behaviour for the water-soluble polymer / surfactant solution from this point onwards will be the same as that of pure surfactant solution.

It has been discovered by this invention that the concentration of the surfactant in the water-soluble polymer / surfactant solution, should be higher than the CAC value of the surfactant in said solution. The preferred amount of surfactant is between the CAC and the CMC value of the surfactant in the water-soluble polymer / surfactant solution itself. More preferably, the amount of the surfactant is equal to or higher than the CMC value. The value for the CAC as well as for CMC are determined herein by a surface tension measurement method known to those skilled in the art.

The suitable surfactant species can be selected from any surfactant that is classified as cationic surfactants, anionic surfactant, non-ionic surfactants or amphoteric surfactants.

Examples of anionic surfactants are including, but not limited to, the fatty acid surfactants such as the regular soaps, phosphate ester surfactants, sulphate ester surfactant such as sodium dodecylsulphate, sulphated fatty acid surfactants such as sulfated monoglycerides and other polyols, and sulphated alkanolamides, sulphated ethers, sulphated alkylphenol ethoxylates, aliphatic sulfonates such as sodium dodecylsulphonate, alkylaryl sulphonates such as sodium dodecyl benzenesulphonate and α-sulphocarboxylic acids and their derivatives.

Examples of suitable cationic surfactants includes the groups containing alkyl nitrogen compounds such as simple ammonium salts containing at least one long chain alkyl group and one or more amine hydrogens, and quartenary ammonium compounds in which all amine hydrogens have been replaced by organic radical substitution, and the groups of cationic surfactants those contain heterocyclic materials characterised by the N-alkylpyridum halides, salts of alkyl-substituted pyridines, morpholinium salts, and imidazolinium derivatives.

The nonionic surfactants include the polyoxy-ethylenes which have the general formula

RX(CH₂CH₂O)ₙH

where R is normally a typical surfactant hydrophobic group, but may also be a polyether such as polyoxypropylene and X is an O, N or another functionality capable of linking the polyoxyethylene chain to the hydrophobe. The "n" represent the average number of the oxyethylene units and should have a value of higher than 5 to impart sufficient water solubility. Another examples of non-ionic surfactants are the derivatives of sugar, derivatives of polyglycerols and other polyols.

The examples of amphoteric surfactants are those categorised as the ampholites such as aminocarboxyclic acids and lecithin, betaines and sulfobetaines.

The selection of the suitable surfactant depends very much on the surface tension of the microporous film itself. In order to have an effective penetration into the pores of the microporous film it is preferred to use a surfactant that has a surface tension value which is equal, more preferably less than the surface tension value of the microporous film. The anionic surfactants including the group of alkylaryl sulphonate such as sodium dodecyl benzene sulphonate, the aliphatic sulfonates such as sodium dodecyl sulphonates and the sulphate ester surfactant such as Aerosil OT have received our preference. The preferred cationic surfactants comprises the groups that contain quartenary ammonium compounds, such as dodecyl trimethyl ammonium chloride.

The amount of water-soluble polymer should preferably be higher than or equal to 0.01 percent weight in order to have significant effect on the increase of the absorption and wettability properties of the treated microporous film. The preferred amount of the water-soluble polymers is preferably equal to or higher than 0.1 weight percent. The viscosity of the solution limits the maximum amount of the water-soluble polymer. It is believed that the viscosity of the solution higher than 50 cP will not effectively penetrate into the pores.

According to this invention, concentration of water-soluble polymer higher than 10 weight percent is usually not favourable since the viscosity of the water-soluble/polymer solution will become too high. However, for some water-soluble polymers which have a low viscosity and/or low gelling point properties such as hydrolysed gelatins and fish gelatins, the maximum concentration may be higher than 10 weight percent.

The water-soluble polymers can be selected from any of the polymers categorised as bio-polymers, synthesis polymers and the mixtures thereof, as long as it is soluble in water. Examples of classes of bio-polymers include protein such as gelatin, casein and other water-soluble protein, dextrin, and starch. The suitable gelatins are in fact those produced from, among others, the bones and skins of animal through the acid or lime treatment, and also those which are modified afterwards through a chemical reaction, enzymatic treatment or heat treatment. Examples of the suitable gelatins are included acid treated pig skin gelatins, acid treated ossein gelatins, lime treated osseïn gelatins, fish skin gelatins, chemically modified gelatins such as modified gelatins with phthalate group, modified gelatins with quartenary ammonium derivatives, modified gelatins with succinyl and dodecenyl succinyl groups, modified gelatin with carbamyl groups, modified gelatin with lauryl groups, modified gelatins with vinyl alcohol groups, modified gelatins with vinyl pyrrolidone, modified gelatins with styrene sulphonate, hydrolysed gelatins and recombinant gelatins. Other examples of the suitable bio-polymers are including starch and starch derivates such as cationic starch, amphoteric starch, oxidized starch, and gum arabic.

There is a lot of variation in the molecular weight of the bio-polymers. An acid or lime bone gelatin for example, has a typical molecular weight in the range of 100 kD to 180 kD. By hydrolysis process, the molecular weight of the lime bone gelatin can be reduced to around 23 kD or even lower when a multiple hydrolysis process is applied to the gelatin. A higher molecular weight gelatin on the other hand, can be produced by a chemical modification of the gelatin itself. According to this invention, the interaction between the water-soluble polymer and the surfactant plays a significant roll. It is believed that a polymer molecule having average molecular weight higher than 200 kD is not suitable for this invention, since the molecules may not efficiently penetrates into the pores. On the other hand, molecular weight of smaller than 1 kD will provide to less interaction with the surfactant molecules. The preferred molecular weight for the bio-polymer is thus between 1kD and 200 kD, more preferably between 5 kD and 50 kD.

Examples of synthetic water-soluble polymers are polyvinyl alcohol, carboxylated polyvinyl alcohol, cellulose derivatives such as polyacryl-amide-hydroxy alkylcellulose, carboxymethylcellulose and hydroxyethylcellulose, hydroxypolyvinyl pyrrolidone, sodium polyacrylate, polyacrylamide, polyamideepichlorohydrin resin, sodium alginate, alkalinically soluble copolymers of styrene and maleic acid anhydride, polyaminoamide resins, polyethyleneoxid, polyethylene imine, quartenary ammoniumsalt polymers, NBR latex, and polyethylene oxide (PEO).

The preferred average molecular weight of the synthetic polymers is in the range of 14 kD to 200 kD.

Depending on the surfactant and the iso-electric point (IEP) of the (bio)-polymer, the suitable pH of the aqueous solution can be determined. The IEP of the (bio)-polymers lies preferably between pH 3.5 and 12.

In order to further improve the wettability and/or the absorption properties as well as the appearance of the microporous film such as whiteness and glossiness, some appropriate additives thereto may be added into the pre-treatment aqueous solution.

For improving the wettability and/or absortivity it is preferably to add hydrophilic particles selected from the non porous colloidal silicious particles, aluminum oxide, calcium carbonate or the mixture thereof. The non-limiting examples of silicious particles are: silica, mica, montmoriillonite, kaolinite, zeolites and aluminum polysilica. Besides the non-poros colloidal particles, the porous particles such as boehmite, pseudo-boehmite, precipitated silica, silica gel, fumed silica or mixture thereof, are also effective for increasing the absorption speed of the ink solvent. The size of the non-porous colloidal particles should be lower than 700 nanometers in order to avoid blocking of the pores of microporous film. The preferred range for the particle size is in between 5 to 100 nm and more preferably between 10 and 70 nm.

For the porous particles, the size of the particles may be somewhat larger than the non-porous colloidal particles since these particles have the ability to absorb the ink solvent. Particle size between 100 to 2000 nm is suitable to be used herein. The suitable pore size of the porous particles should be in the range of 1 and 500 nm.

The maximum amount of the particles in the water-soluble polymer / surfactant is mainly determined by the final viscosity of the solution. Depending on the charges of the water-soluble polymer, the surfactant and the particles, some degree of interaction between those three components may be expected. This interaction may result in a high solution viscosity, which is not favourable for this invention. Additive particles' amount higher than 50 weight percent of the aqueous solution is thought to be not practical. The suitable amount should be lower than 45 weight percent. The preferred amount for the particles is lower than 35 weight percent and it is more preferable to have a concentration in the range of 1 and 30 weight percent.

The thermoplastic polymers suitable for manufacturing the microporous film are available in a huge number and kinds. In general, any substantially water-insoluble thermoplastic polymers, that can be extruded, calandered, pressed or rolled into film, sheet, strip or web may be used.

The polymer resin is stretched after production. This can be done in the conventional way. The stretching may be monoaxially or biaxially. Generally the degree of stretching is such that it the required pore volume is obtained.

The polymer may be a single polymer or a mixture of polymers. The polymers may be homopolymers, copolymers, random polymers, block copolymers, atactic polymers, isotactic polymers, syndiotactic polymers, linear polymers, or branched polymers. When mixtures of polymers are used, the mixtures may be homogeneous, or it may comprise two or more polymeric phases. Examples of classes of suitable thermoplastic polymers include the polyolefins, poly(halo-substituted polyolefins), polyesters, polyamides, polyurethans, polyureas, polystyrene, poly(vinyl-halides), poly (vinylidene halides), polystyrenes, poly(vinyl esters), polycarbonates, polyethers, polysulfides, polyimides, polysilanes, polysiloxanes, polycaprolactames, polyacrylates, and polymethacrylates. Examples of suitable thermoplastic polymers include high density polyethylene, low density polyethylene, ultra high molecular weight polyethylene, polypropylene (atactic, isotactic or syndiotic), poly(vinyl chloride), polytetrafluroethylene, copolymers of ethylene and alpha-olefines, copolymers of ethylene and acrylic acids, copolymers of ethylene and methacrylic acids, copolymers of ethylene and vinyl acetate, copolymers of propylene and alpha-olefines, poly(vinylidene chloride), copolymers of vinylidene chloride and vinyl acetate, copolymers of vinylidene chloride and vinyl chloride, copolymers of ethylene and propylene, copolymers of ethylene and butene, poly(vinyl acetate), polystyrene, poly(omega-aminoundecanoic acid), poly(-methyl methacrylate), poly(hexamethylene adipamide), poly(epsilon- caprolactam).

The preferred thermoplastics are polyolefin comprising polyethylene, polypropylene, co-polymers of ethylene and alpha-olefines, vinyl ethylene-acetate co-polymers, methyl ethylene-acrylate co-polymers, ethyl ethylene-acrylate co-polymers, acrylic ethylene-acid co-polymers and the ionomers or the mixture thereof.

The fillers can be selected either from the groups of organic fillers and inorganic fillers. The examples of organic fillers include wood particles, pulp particles, cellulose type particles, polymer particles such as Teflon TM particles and Kevlar TM particles, nylon particles dispersed in polypropylene, polybutylene terephthalate particles in polypropylene, and polypropylene dispersed in polyethylene terephthalate. The important characteristics of these organic fillers are it size and the shape of the particles. Spheres are preferred and they can be hollow or solid.

Examples of the inorganic fillers are included the groups consisting of calcium carbonate, clay, silica, titanium dioxide, talc, clay, kaoline, magnesium sulphate, barium sulphate, calcium sulphate, aluminum hydroxide, magnesium hydroxide, calcium hydroxide, magnesium oxide, zinc oxide, zeolite. The preferred filler is calcium carbonate, silica barium sulphate, titanium dioxide or mixture thereof, having particle sizes lower than 40 µm, preferably in the range of 0.5 and 10 µm.

The amount of filler added to the polyolefin depends on the desired properties of the microporous film including tear strength, water vapour transmission rate and stretchability. It is believed that the voids volume created in the microporous film can not be reached sufficiently for the invention mentioned herein with an amount of filler less than about 30 percent by weight. The more we are able to increase the filler loading amount, the more suitable the film will be due to the increase of the void volume. In order to obtain a filler loading higher than 80 weight percent in the polymer, it may be necessary to coat the inorganic filler with fatty acids such as fatty acid ester, silicone oil or silanes.

In this invention, the microporous film is adhered on a support 14 through an adhesive layer 13, as it is illustrated in figure 1. As it is mentioned previously pre-treatment solution can be applied either before or after lamination process of the microporous film. The adhesive layer 13, can be of any materials that have a good properties for adhering the microporous film 11 on the support 14. Examples of such materials are included polyolefin such as polyethylen and polypropylene, polyesthers, polyamide, starch, gelatin, gums arabic, pectin, albumin and agar-agar. More preferable materials for the adhesive layer 13 are those which are permeable to various gas, especially to air and water vapour. The examples of the preferred materials for the adhesive layer is included starch, gelatin, pectin, gum arabic, albumin and agar-agar.

The support 14 is preferably coated on the back side with a polymer matrix comprises of at least a polyolefin resin and an anti-static agent. This back coating is illustrated in figure 1 as the layer 15. Furthermore, the support is selected from a photographic base paper, a synthetic paper or a plastic film.

Examples of the material of the plastic film are polyolefins such as polyethylene and polypropylene, vinyl copolymers such as polyvinyl acetate, polyvinyl chloride and polystyrene, polyamide such as 6,6-nylon and 6-nylon, polyesters such as polyethylene terephtalate, polyethylene-2 and 6-naphtalate and polycarbonate, and cellulose acetates such as cellulose triacetate and cellulose diacetate.

The ink receiving layer 12 is characterised by the hygroscopic properties of said layer and its high ability to fix the image with a precise dot size and to provide good image stability. The said ink receiving layer comprises binders, fine porous pigments particles selected from the groups of aluminum oxides such as boehmite and pseudo-boehmite and those of silica such as silica gel and precipitated silica, and optionally various known additives, including surfactants, dye-fixing agent, mordant, etc. Optionally the ink receiving layer 12 may comprise other materials to improve the whiteness and the glossiness appearances of the ink jet medium 10. As the binder, it is usually possible to employ an organic material such as gelatin or one of its modified products, poly (vinyl alcohol), NBR latex, cellulose derivatives, quartenary ammonium salt polymers poly vinyl pyrrolidone or other suitable binders.

In order to further improve the gloss appearance and other additional properties, we may coat an over-coating layer 26, as illustrated in figure 2, on top of the ink receiving layer. This layer may comprise cellulose derivatives such as hydroxymethyl cellulose and hydroxyethyl cellulose, polyvinyl alcohol or gelatin in combination with a suitable cross-linking agent. The over coating layer is non-porous but is ink permeable.

### Examples

The present invention will be explained in detail by the following non-limiting examples.

### Example 1.

The aqueous impregnation solution is prepared by solving 1 weight percent of a hydrolysed lime bone gelatin (GEL-1) having an iso-electric point around pH 5.2, average MW around 23 KD, in water by swelling the gelatin particles for 15 minutes and dissolving the swollen gelatin at temperature of 40°C. The solution is then coated on an ACE microporous film type 949, purchased from ACE S.A. (Belgium), by using a RK grooved bar coater #2. The ACE film is attached to a normal copying paper prior to coating. The coated solution is dried at room temperature and thereafter the contact angle as well as the absorption speed of 1 µl water drop on the pre-treated ACE film, by using the VCA contact angle apparatus made by AST Product, Inc. (USA). The Software of the VCA, VCA 2500, records the changes of the contact angle as well as the volume of the drop for 10 seconds with a recording speed of 4 images per seconds. The absorbed volume as function of time is then calculated by simply extracting the initial volume of drops with the remaining volume of the drop. The result of the measurements is given in table 1.

### Example 2

Another aqueous impregnation solution is prepared by solving 2 weight percent of GEL-1 according to the procedure mentioned in example 1. Into the 2wt.% gelatin solution, some amount of an-ionic surfactant sodium dodecyl benzene sulphonate (SDBS, MW= 348.49), obtained from ICN Biochemicals, Inc. (USA), is added into the gelatin solution in such away that the final solution is containing 1wt% GEL-1 solution and 1 mmol/L SDBS.

This aqueous solution is then coated on the ACE film type 949 according to the procedure mentioned in example 1. After drying, the contact angle as well as the absorption speed of 1 µl water drop on the pre-treated ACE film are measured, using the VCA contact angle apparatus. The result of the measurements is given in table 1.

### Example 3

The ACE 949 film is impregnated with an aqueous solution containing 1 wt% GEL-1 and 50 mmol/L SBDS as in example 2. The result of the contact angle and absorption speed measurement is given in table 1.

### Comparative example 1

The contact angle of 1 µl water drop as well as the absorption speed of 1 µl water drop on the untreated ACE film are measured by the method described in example 1.

**Table 1.**

| | SDBS conc. [mmol/L] in 1 wt.% GEL-1 solution | Contact angle | | Absorption speed [µL/s.] |
|---|---|---|---|---|
| | | t=0 s | t= 10 s | |
| Ex. 1 | 0 (=pure GEL-1 sol.) | 75° | 31° | 0.22 |
| Ex.2 | 1 | 68° | 39° | 0.30 |
| Ex.3 | 50 | 48° | 17° | 0.47 |
| Comp. Ex.1 | untreated ACE film | 108° | 108° | 0.001 |

### Example 4

Into a 100 mmol/L SDBS solution in water, a GEL-2 solution is added in such a way that the final concentration of SDBS and GEL-2 in the solution is respectively 60 mmol/L and 1 wt%. The temperature of the solution is kept at 40°C. The gelatin GEL-2 is a lime bone gelatin having an IEP around pH 5.0 and MW around 160 KD.
The ACE 949 film is then impregnated with this solution according to example 1. The contact angle and absorption speed of the treated ACE film towards water drops is measured according to the method mentioned in example 1, and the results are given in table 2.

### Example 5

Example 4 is repeated by using GEL-3 solution in stead of GEL-2. The GEL-3 is a phthalated lime bone gelatin having an IEP around pH 3.8 and having average MW around 180 KD. The results of the contact angle and absorption speed measurement can be found in table 2.

### Example 6

Example 4 is repeated by using GEL-4 solution in stead of GEL-2. GEL-4 is an acid pigskin gelatin having an IEP around pH 9.0 and having average MW around 130 KD. The results of the contact angle and absorption speed measurement can be found in table 2.

### Example 7

Example 4 is repeated by using polyvinyl alcohol (PVA) solution in stead of GEL-2 at room temperature. The PVA is the Mowiol 23-88, purchased from Clariant GmbH , Frankfurt, Germany. The hydrolyses grade of the PVA is 87.7 mol%. The results of the contact angle and absorption speed measurement can be found in table 2.

### Example 8

Example 4 is repeated by using GEL-1 solution. For this experiment, 50 mmol/L dodecyl trimethyl ammonium chloride (DTMAC) is used as surfactant in stead of SDBS. The DTMAC solution of 50weight percent, is obtained from ICN Biomedicals Inc. The results of the contact angle and absorption speed measurement can be found in table 2.

### Example 9

The same experiment as ex. 8 is prepared for GEL-4 solution. Next to the DTMA.C, a 50wt% Sylojet® A200 solution is added into the gelatin solution. The Sylojet® A200 solution contained about 20 wt% Al₂O₃ and is purchased from Grace Davidson Inc, (USA). The results of the contact angle and absorption speed measurement can be found in table 2.

**Table 2**

| | Water-soluble polymer. [1 wt.%] in 50 mmol/L SDBS | Contact angle | | Absorption speed [µL/s.] |
|---|---|---|---|---|
| | | t = 0 s | t = 10 s | |
| Ex. 4 | GEL-2 | 49° | 21° | 0.65 |
| Ex. 5 | GEL-3 | 51° | 26° | 0.79 |
| Ex. 6 | GEL-4 | 45° | 19° | 0.71 |
| Ex. 7 | Mowiol 23-88 | 55° | | 0.50 |
| Ex. 8 | GEL-1 + 50 mmol/L DTMAC | 47° | 19° | 0.98 |
| Ex. 9 | GEL-4 + 50 mmol/L DTMAC +A200 | 27° | 19° | 1.46 |

### Example 10

Another set of experiments was done, analyzing the effect of impregnation solution on the drying speed of the ink jet media. An ACE microporous films is adhered onto a 166 gr/m² paper base by means of an adhesive layer containing phtalated lime bone gelatin (GEL-3) and silica gel (Sylojet 703 A, from Grace Davidson, USA). The dry solid content ratio between the GEL-3 and Silica gel is 1 to 2. The surface tension of the ACE film is measured by the contact angle method known in the field of art and is amounted 30-38 dyne/cm.

The impregnation solution is prepared by mixing the solutions of 2 wt% GEL-5 with 2wt% Aerosol OT (Nippon Yushi, Japan) and de-ionized water in such away that the final concentration of the GEL-5 and Aerosol OT is respectively 1wt% and 0.8 wt%. The gelatin GEL-5 is a hydrolyzed lime gelatin having an IEP around pH 5.2 and MW around 1.5 to 2 KD. The surface tension of 1wt% Aerosol OT in water is 25 dyne/cm.

The ink receiving solution is prepared by mixing 615 parts of 28.6 wt% of HP-14 sol, 275 parts of 10wt% of PVA Mowiol 23-88 (purchased from Clariant), and 110 parts of de-ionized water. The HP-14 powder contains alumina hydrate of boehmite structure and is purchased from Sasol, Germany.

### Impregnation and coating the adhered microporous film

The ACE film is treated with the impregnation solution by using a RK grooved bar #3 and dried at room temperature for about 3 hours. Thereafter, the ink receiving solution is coated on the impregnated ACE film by using a RK grooved bar # 5 and dried at 70C for about 2 hours.

### Printing test:

The microporous ink jet media is further subjected to an ink-jet printing test. A standard pattern comprising the colours magenta, cyan, yellow, green, red, blue and black in 5 different densities is printed on the above mentioned microporous substrates. The printers which were used herein are Epson PM 770C and HP 990.

Directly after printing the standard pattern, a white paper was overlaid on the printed microporous substrate and a stainless steel roller with a weight of 10 kg was rolled over the white paper slowly. The drying speed of the microporous substrate was determined by analyzing visually the colour density of the print which was transferred to the white paper. A lower density at the white paper means a better drying speed of the ink jet solvent. The results of the printing test can be found in table 3.

### Example 11

The same experiment as mentioned in Example 10 is conducted, except that GEL-6 is used in the impregnation solution in stead of GEL-5. The GEL-6 is a lime bone gelatin having average MW of 160 kD and an IEP around pH 5. The result of the printing test can be found in table 3.

### Comparative Example 2

The same experiment as mentioned in Example 10 is carried out, except that the impregnation solution contains only 1 wt% Aerosol OT. The result of the printing test can be found in table 3.

### Comparative example 3

The similar experiment as mentioned in Example 10 is carried out. In this test the microporous film is not impregnated. It is directly coated with the said ink receiving layer. The result of the printing test is listed in table 3.

**Table 3**

| | Impregnation solution | Drying speed*) | |
|---|---|---|---|
| | | Epson 770C | HP990 |
| Ex. 10 | 1 wt.% GEL-5 and 0.8wt.% Aerosol OT. GEL-5: MW = 1.5 - 2 KD | O | O |
| | Surface tension 1wt% Aerosol OT in water at 20C : 25 dyne/cm | | |
| Ex. 11 | 1 wt.% GEL-6 and 0.8 wt.% Aerosol OT. GEL-6: MW = 160 KD | Δ | Δ |
| Comp. Ex. 2 | Only 1wt% Aerosol OT | X | Δ - X |
| Comp. Ex. 3 | No impregnation | XX | XX |

| | | | |
|---|---|---|---|
| *) Definitions: O = Good Δ = Not totally dry but still acceptable X = Bad (not acceptable) XX = Very bad and causing serious colour bleeding | | | |

From these experiments it can be seen that the formulation of impregnation solution has a significant effect on the drying speed of the print.

## Claims

1. An ink jet recording medium comprising:
- a support,
- a water-repellent microporous film adhered to said support, said microporous film being an oriented thermoplastic film comprising fillers and having interconnecting channels between the pores, with a void volume between 30 to 90 volume percent of the total microporous film, wherein said microporous film has been impregnated with an aqueous solution comprising at least a water-soluble polymer and surfactant,
- at least one ink receiving layer as a coating on said impregnated microporous film, and optionally,
- a protective layer on top of the ink receiving layer.

2. The medium according to claim 1, wherein the thickness of said microporous film is less than 150 micrometers.

3. The medium according to claim 1 or 2, wherein the thickness of said microporous film is between 15 to 100 micrometers.

4. The medium according to claim 1-3, wherein the amount of said water-soluble polymer is at least 0.01 weight percent of the aqueous solution.

5. The medium according to claim 1-4, wherein the amount of surfactant in the aqueous solution is higher than the critical aggregation concentration (CAC) of the surfactant / water-soluble polymer solution itself.

6. The medium according to claim 5, wherein the amount of surfactant in the aqueous solution is between the critical aggregation concentration (CAC) and the critical micelle concentration (CMC) of the surfactant / water-soluble polymer solution itself.

7. The medium according to claim 5, wherein the amount of the surfactant is equal to or higher than the critical micelle concentration (CMC) of the surfactant / water-soluble polymer solution.

8. The medium according to claim 1-7, wherein the viscosity of the aqueous solution during treatment of the microporous film is lower than 50 cP.

9. The medium according to claim 1-8, wherein the water-soluble polymer is chosen from the group of material consisting of gelatin, phthalated gelatin, modified gelatin with ammonium derivatives, modified gelatin with succinyl groups, modified gelatin with vinyl alcohol groups, modified gelatin with vinyl pyrrolidone groups, hydrolised gelatin, polyvinyl alcohol (PVA), polyvinyl pyrrolidone (PVP), polyethylene oxide (PEO), polyacryl amide, polyacrylate and mixtures thereof.

10. The medium according to claim 9, wherein the water-soluble polymer comprises gelatin, polyvinyl alcohol (PVA), polyvinyl pyrrolidone (PVP), polyethylene oxide (PEO) or mixtures thereof.

11. The medium according to claim 1-10, wherein the water-soluble polymer comprises gelatin with an average molecular weight between 1 kD to 200 kD, or polyvinyl alcohol (PVA), polyvinyl pyrrolidone (PVP), polyethylene oxide (PEO) or mixtures of the synthetic polymers having an average molecular weight between 14 kD and 200 kD.

12. The medium according to claim 11, wherein the water-soluble polymer comprises gelatin with an average molecular weight between 1 kD to 50 kD, or polyvinyl alcohol (PVA), polyvinyl pyrrolidone (PVP), polyethylene oxide (PEO) or mixtures of the synthetic polymers having an average molecular weight between 60 kD and 180 kD.

13. The medium according to claim 1-12, wherein the iso-electric point (IEP) of said water-soluble polymer is in the range of pH 3.5 and 12.

14. The medium according to claim 1-13, wherein the surfactant is selected from the group of anionic surfactants, cationic, non-ionic and amphoteric surfactants.

15. The medium according to claim 14, wherein the surfactant is selected from the anionic surfactants containing alkylaryl sulphonates, sulphate ester and aliphatic sulphonates, and from the cationic surfactants containing quarternary ammonium compounds.

16. The medium according to claim 1-15, wherein the aqueous solution further contains additives in an amount lower than 45 weight percent of the aqueous solution.

17. The medium according to claim 16, wherein the amount of additives is lower than 35 weight percent of the aqueous solution.

18. The medium according to claims 16 or 17, wherein the amount of additives is in the range between 1 and 30 weight percent of the aqueous solution.

19. The medium according to any of the claims 16-18, wherein said additives comprise non-porous colloidal particles selected from the group consisting of silicious particles, aluminum oxide and calcium carbonate, or porous particles including boehmite, pseudo-boehmite, precipitated silica, silica gel and fumed silica, and mixtures thereof.

20. The medium according to claim 19, wherein the size of said colloidal particles is in the ranges between 5 to 700 nm.

21. The medium according to claim 20, wherein the size of said colloidal particles is in the ranges between 5 to 100 nm.

22. The medium according to claim 21, wherein the size of said colloidal particles is in the ranges between 5 to 70 nm.

23. The medium according to claim 19-22, wherein said additives comprising porous particles having an average particle size in the range between 100 and 2000 nanometers.

24. The medium according to claim 23, wherein the size of the pores of said porous particles are in the range between 1 and 500 nanometers.

25. The medium according to claim 1-24, wherein said microporous film is obtainable by a manufacturing process comprising mixing of an orientable thermoplastic resin with at least one coated filler, extruding said mixture at elevated temperatures to form a film thereof, pre-stretching the film, cooling said film until the film is solidified and stretching said cooled film to form a microporous film.

26. The medium according to claim 1-25, wherein said microporous film comprises of 30 to 90 weight percent of filler.

27. The medium according to claim 1-26, wherein said filler comprises calcium carbonate, barium sulphate, silica, titanium dioxide or a mixture thereof.

28. The medium according to claim 1- 27, wherein said filler has an average particle size less than 40 µm.

29. The medium according to claim 28, wherein said filler has an average particle size preferably between 0.5 µm and 10 µm.

30. The medium according to claim 25- 29, wherein the thermoplastic resin comprises polyethylene, polypropylene, co-polymers of ethylene and alphaolefins, co-polymers of ethylene and acrylic acids, copolymers of ethylene and methacrylic acids, copolymers of ethylene and vinyl acetate, copolymers of propylene and alpha-olefines, poly(vinylidene chloride), copolymers of vinylidene chloride and vinyl acetate, copolymers of vinylidene chloride and vinyl chloride, copolymers of ethylene and propylene, copolymers of ethylene and butene, poly(vinyl acetate), polystyrene, poly(omega-aminoundecanoic acid), poly(-methyl methacrylate), poly(hexamethylene adipamide), and/or poly(epsilon- caprolactam).

31. Medium according to claim 30, wherein the thermoplastic resin comprises polyethylene; polypropylene; co-polymers of ethylene and alpha-olefines; vinyl ethylene-acetate, co-polymers methyl ethylene-acrylate co-polymers ethyl ethylene-acrylate co-polymers, acrylic ethylene-acid co-polymers; and the ionomers, or the mixture thereof.

32. The medium according to claim 1-31, wherein said support is a photographic base paper, a synthetic paper or a film substrate.

33. The medium according to claim 1-32, wherein said support is laminated on one side with a polymer matrix comprising at least a polyolefin resin.

34. The medium according to claim 1-33, wherein said ink receiving layer comprises absorbent particles and binder.

35. The medium according to claim 34, wherein said absorbent particles in the ink receiving layer is silica, boehmite, pseudo boehmite or combination thereof.

36. The medium according to claim 34 or 35, wherein said binder in the ink receiving layer comprises gelatins, polyvinyl alcohol, polyvinyl pyrolidone, cellulose derivatives or the mixtures thereof.

37. The medium according to claim 1-36, further comprising an ink-permeable protective layer on top of said ink receiving layer.

38. The medium according to claim 37, wherein said protective layer comprises hydroxypropyl methyl cellulose, polyvinyl alcohol or gelatin solution.

39. Method for preparing an ink jet recording medium comprising the steps of:
a. pre-treating a water-repellent microporous film with an aqueous solution comprising at least a water-soluble polymer and surfactant, said microporous film being an oriented thermoplastic film comprising fillers and having interconnecting channels between the pores, with a void volume between 30 to 90 volume percent of the total microporous film;
b. adhering said film to a support;
c. coating an ink receiving layer on said film; optionally followed by
d. coating a protective layer on top of said ink receiving layer; wherein step a is carried out before step c.

40. Method according to claim 39, wherein step a is carried out before step b.

41. A method of forming a permanent, precise ink jet image comprising the step of:
providing an ink jet recording medium according to any one of the claims 1-38 introducing ink jet ink into contact with the medium in the pattern of a desired image.

42. A hydrophilic and hygroscopic microporous film, which is obtainable by impregnating a water repellent film comprising an oriented thermoplastic and at least one filler, which film is permeable to air and water vapour, and has a void volume between 30 and 90 volume percent of the total film, with an aqueous solution comprising at least a water-soluble polymer and surfactant.

## Patentansprüche

1. Tintenstrahl-Aufzeichnungsmedium, das umfasst:
- einen Träger,
- einen an dem Träger haftenden wasserabstoßenden mikroporösen Film, bei dem es sich um einen orientierten thermoplastischen Film handelt, der Füllstoffe umfasst und Verbindungskanäle zwischen den Poren aufweist mit einem Hohlraumvolumen zwischen 30 und 90 Vol.-% des gesamten mikroporösen Films, wobei der mikroporöse Film mit einer wässrigen Lösung imprägniert ist, die mindestens ein wasserlösliches Polymer und ein Tensid umfasst,
- mindestens eine Tinte aufnehmende Schicht als Überzug auf dem imprägnierte mikroporösen Film und gegebenenfalls
- eine Schutzschicht auf der Oberseite der Tinte aufnehmenden Schicht.

2. Medium nach Anspruch 1, in dem die Dicke des mikroporösen Films weniger als 150 µm beträgt.

3. Medium nach Anspruch 1 oder 2, in dem die Dicke des mikroporösen Films zwischen 15 und 100 µm liegt.

4. Medium nach den Ansprüchen 1 bis 3, in dem die Menge des wasserlöslichen Polymers mindestens 0,01 Gew.%, bezogen auf das Gewicht der wässrigen Lösung, beträgt.

5. Medium nach den Ansprüchen 1 bis 4, in dem die Menge des Tensids in der wässrigen Lösung höher ist als die kritische Aggregationskonzentration (CAC) der Tensid/wasserlöslichen Polymer-Lösung selbst.

6. Medium nach Anspruch 5, in dem die Menge des Tensids in der wässrigen Lösung zwischen der kritischen Aggregationskonzentration (CAC) und der kritischen Micellenkonzentration (CMC) der Tensid/wasserlöslichen Polymerlösung selbst liegt.

7. Medium nach Anspruch 5, in dem die Menge des Tensids gleich oder höher ist als die kritische Micellenkonzentration (CMC) der Tensid/wasserlöslichen Polymer-Lösung.

8. Medium nach den Ansprüchen 1 bis 7, in dem die Viskosität der wässrigen Lösung während der Behandlung des mikroporösen Films weniger als 50 cP beträgt.

9. Medium nach den Ansprüchen 1 bis 8, in dem das wasserlösliche Polymer ausgewählt ist aus einer Gruppe von Materialien, die besteht aus Gelatine, phthalalierter Gelatine, modifizierter Gelatine mit Ammonium-Derivaten, modifizierter Gelatine mit Succinylgruppen, modifizierter Gelatine mit Vinylalkoholgruppen, modifizierter Gelatine mit Vinylpyrrolidongruppen, hydrolysierter Gelatine, Polyvinylalkohol (PVA), Polyvinylpyrrolidon (PVP), Polyethylenoxid (PEO), Polyacrylamid, Polyacrylat und Mischungen davon.

10. Medium nach Anspruch 9, in dem das wasserlösliche Polymer Gelatine, Polyvinylalkohol (PVA), Polyvinylpyrrolidon (PVP), Polyethylenoxid (PEO) oder Mischungen davon umfasst.

11. Medium nach den Ansprüchen 1 bis 10, in dem das wasserlösliche Polymer Gelatine mit einem durchschnittlichen Molekulargewicht zwischen 1 und 200 kD oder Polyvinylalkohol (PVA), Polyvinylpyrrolidon (PVP), Polyethylenoxid (PEO) oder Mischungen der synthetischen Polymeren mit einem durchschnittlichen Molekulargewicht zwischen 14 und 200 kD umfasst.

12. Medium nach Anspruch 11, in dem das wasserlösliche Polymer Gelatine mit einem durchschnittlichen Molekulargewicht zwischen 1 und 50 kD oder Polyvinylalkohol (PVA), Polyvinylpyrrolidon (PVP), Polyethylenoxid (PEO) oder Mischungen der synthetischen Polymeren mit einem durchschnittlichen Molekulargewicht zwischen 60 und 180 kD umfasst.

13. Medium nach den Ansprüchen 1 bis 12, in dem der isoelektrische Punkt (IEP) des wasserlöslichen Polymers in dem Bereich von pH 3,5 bis 12 liegt.

14. Medium nach den Ansprüchen 1 bis 13, in dem das Tensid ausgewählt ist aus der Gruppe, die besteht aus anionischen Tensiden, kationischen, nicht-ionischen und amphoteren Tensiden.

15. Medium nach Anspruch 14, in dem das Tensid ausgewählt ist aus den anionischen Tensiden, die Alkylarylsulfonate, Sulfatester und aliphatische Sulfonate enthalten, und aus den kationischen Tensiden, die quaternäre Ammonium-Verbindungen enthalten.

16. Medium nach den Ansprüchen 1 bis 15, in dem die wässrige Lösung außerdem Additive in einer Menge von weniger als 45 Gew.-%, bezogen auf das Gewicht der wässrigen Lösung, enthält.

17. Medium nach Anspruch 16, in dem die Menge der Additive weniger als 35 Gew.-%, bezogen auf das Gewicht der wässrigen Lösung, beträgt.

18. Medium nach Anspruch 16 oder 17, in dem die Menge der Additive in dem Bereich zwischen 1 und 30 Gew.%, bezogen auf das Gewicht der wässrigen Lösung, liegt.

19. Medium nach einem der Ansprüche 16 bis 18, in dem die Additive umfassen nicht-poröse kolloidale Teilchen, ausgewählt aus der Gruppe, die besteht aus Siliciumdioxid-haltigen Teilchen, Aluminiumoxid und Calciumcarbonat, oder poröse Teilchen einschließlich Boehmit, Pseudoboehmit, präzipitiertes Siliciumdioxid, Silicagel und abgerauchtem Siliciumdioxid und Mischungen davon.

20. Medium nach Anspruch 19, in dem die Größe der kolloidalen Teilchen in dem Bereich zwischen 5 und 700 nm liegt.

21. Medium nach Anspruch 20, in dem die Größe der kolloidalen Teilchen in dem Bereich zwischen 5 und 100 nm liegt.

22. Medium nach Anspruch 21, in dem die Größe der kolloidalen Teilchen in dem Bereich zwischen 5 und 70 nm liegt.

23. Medium nach Anspruch 19 bis 22, in dem die Additive poröse Teilchen mit einer durchschnittlichen Teilchengröße in dem Bereich zwischen 100 und 2000 nm umfassen.

24. Medium nach Anspruch 23, in dem die Größe der Poren der porösen Teilchen in dem Bereich zwischen 1 und 500 nm liegt.

25. Medium nach den Ansprüchen 1 bis 24, in dem der mikroporöse Film erhältlich ist durch ein Herstellungsverfahren, das umfasst
das Vermischen eines orientierbaren thermoplastischen Harzes mit mindestens einem beschichteten Füllstoff,
das Extrudieren der Mischung bei erhöhten Temperaturen zur Bildung eines Films daraus,
das Vorverstrecken des Films,
das Abkühlen des Films, bis der Film erstarrt ist, und Verstrecken des abgekühlten Films zur Bildung eines mikroporösen Films.

26. Medium nach den Ansprüchen 1 bis 25, in dem der mikroporöse Film 30 bis 90 Gew.-% Füllstoff umfasst.

27. Medium nach den Ansprüchen 1 bis 26, in dem der Füllstoff Calciumcarbonat, Bariumsulfat, Siliciumdioxid, Titandioxid oder eine Mischung davon umfasst.

28. Medium nach den Ansprüchen 1 bis 27, in dem der Füllstoff eine durchschnittliche Teilchengröße von weniger als 40 µm aufweist.

29. Medium nach Anspruch 28, in dem der Füllstoff eine durchschnittliche Teilchengröße aufweist, die vorzugsweise zwischen 0,5 und 10 µm liegt.

30. Medium nach den Ansprüchen 25 bis 29, in dem das thermoplastische Harz Polyethylen, Polypropylen, Copolymere von Ethylen und α-Olefinen, Copolymere von Ethylen und Acrylsäuren, Copolymere von Ethylen und Methacrylsäuren, Copolymere von Ethylen und Vinylacetat, Copolymere von Propylen und α-Olefinen, Poly(vinylidenchlorid), Copolymere von Vinylidenchlorid und Vinylacetat, Copolymere von Vinylidenchlorid und Vinylchlorid, Copolymere von Ethylen und Propylen, Copolymere von Ethylen und Buten, Poly(vinylacetat), Polystyrol, Poly(ω-aminoundecansäure), Poly(methylmethacrylat), Poly(hexamethylenadipamid) und/oder Poly(ε-caprolactam) umfasst.

31. Medium nach Anspruch 30, in dem das thermoplastische Harz Polyethylen; Polypropylen; Copolymere von Ethylen und α-Olefinen; Vinylethylen-Acetat-Copolymere, Methylethylen-Acrylat-Copolymere, Ethylethylen-Acrylat-Copolymere, Acryl-Ethylen-Säure-Copolymere und lonomere oder eine Mischung davon umfasst.

32. Medium nach den Ansprüchen 1 bis 31, in dem der Träger ein fotografisches Trägerpapier, ein synthetisches Papier oder ein Filmsubstrat ist.

33. Medium nach den Ansprüchen 1 bis 32, in dem auf eine Seite des Trägers eine Polymermatrix auflaminiert ist, die mindestens ein Polyolefinharz umfasst.

34. Medium nach den Ansprüchen 1 bis 33, in dem die Tinte aufnehmende Schicht absorptionsfähige Teilchen und ein Bindemittel umfasst.

35. Medium nach Anspruch 34, in dem die absorptionsfähigen Teilchen in der Tinte aufnehmenden Schicht Siliciumdioxid, Boehmit, Pseudoboehmit oder eine Kombination davon sind.

36. Medium nach Anspruch 34 oder 35, in dem das Bindemittel in der Tinte aufnehmenden Schicht Gelatine, Polyvinylalkohol, Polyvinylpyrrolidon, CelluloseDerivate oder Mischungen davon umfasst.

37. Medium nach den Ansprüchen 1 bis 36, das außerdem eine für Tinte durchlässige Schutzschicht auf der Oberseite der Tinte aufnehmenden Schicht umfasst.

38. Medium nach Anspruch 37, in dem die Schutzschicht Hydroxypropylmethylcellulose, Polyvinylalkohol oder eine Gelatinelösung umfasst.

39. Verfahren zur Herstellung eines Tintenstrahl-Aufzeichnungsmediums, das die Stufen umfasst:
a. Vorbehandeln eines wasserabstoßenden mikroporösen Films mit einer wässrigen Lösung, die mindestens ein wasserlösliches Polymer und ein Tensid umfasst, wobei der mikroporöse Film ein orientierter thermoplastischer Film ist, der Füllstoffe umfasst und Verbindungskanäle zwischen den Poren aufweist mit einem Hohlraumvolumen zwischen 30 und 90 Vol.-% des gesamten mikroporösen Films;
b. haftendes Verbinden des Films mit einem Träger;
c. Aufbringen einer Tinte aufnehmenden Schicht auf den Film; woran sich gegebenenfalls anschließt
d. das Aufbringen einer Schutzschicht auf die Oberseite der Tinte aufnehmenden Schicht;
wobei die Stufe (a) vor der Stufe (c) durchgeführt wird.

40. Verfahren nach Anspruch 39, worin die Stufe (a) vor der Stufe (b) durchgeführt wird.

41. Verfahren zur Erzeugung eines dauerhaften scharfen Tintenstrahl-Aufzeichnungsbildes, das die Stufe umfasst:
Bereitstellen eines Tintenstrahl-Aufzeichnungsmediums nach einem der Ansprüche 1 bis 38 und Inkontaktbringen der Tintenstrahltinte mit dem Medium in Form eines gewünschten Bildmusters.

42. Hydrophiler und hygroskopischer mikroporöser Film, der erhältlich ist durch Imprägnieren eines wasserabstoßenden Films, der einen orientierten thermoplastischen Kunststoff und mindestens einen Füllstoff umfasst, wobei der Film für Luft und Wasserdampf durchlässig ist und ein Hohlraumvolumen zwischen 30 und 90 Vol.-%, bezogen auf den gesamten Film, aufweist, mit einer wässrigen Lösung, die mindestens ein wasserlösliches Polymer und ein Tensid umfasst.

## Revendications

1. Milieu d'enregistrement pour jet d'encre comprenant :
- un support,
- un film microporeux hydrofuge adhérant audit support, ledit film microporeux étant un film thermoplastique orienté comprenant des charges et comportant des canaux d'interconnexion entre les pores, avec un volume de vide compris entre 30% et 90% en volume de l'ensemble du film microporeux, dans lequel ledit film microporeux est imprégné d'une solution aqueuse comprenant au moins un polymère hydrosoluble et un tensio-actif,
- au moins une couche réceptrice d'encre en tant que revêtement sur ledit film microporeux imprégné et, éventuellement,
- une couche protectrice par-dessus la couche réceptrice d'encre.

2. Milieu selon la revendication 1, dans lequel l'épaisseur dudit film microporeux est inférieure à 150 micromètres.

3. Milieu selon la revendication 1 ou 2, dans lequel l'épaisseur dudit film microporeux est comprise entre 15 et 100 micromètres.

4. Milieu selon les revendications 1 à 3, dans lequel la quantité dudit polymère hydrosoluble est d'au moins 0,01% en poids de la solution aqueuse.

5. Milieu selon les revendications 1 à 4, dans lequel la quantité de tensio-actif dans la solution aqueuse est supérieure à la concentration d'agrégation critique (CAC) de la solution tensio-actif/polymère hydrosoluble elle-même.

6. Milieu selon la revendication 5, dans lequel la quantité de tensio-actif dans la solution aqueuse est comprise entre la concentration d'agrégation critique (CAC) et la concentration micellaire critique (CMC) de la solution tensio-actif/polymère hydrosoluble elle-même.

7. Milieu selon la revendication 5, dans lequel la quantité de tensio-actif est égale ou supérieure à la concentration micellaire critique (CMC) de la solution tensio-actif/polymère hydrosoluble.

8. Milieu selon les revendications 1 à 7, dans lequel la viscosité de la solution aqueuse pendant le traitement du film microporeux est inférieure à 50 cP.

9. Milieu selon les revendications 1 à 8, dans lequel le polymère hydrosoluble est choisi dans le groupe de matières constitué par la gélatine, la gélatine phtalatée, la gélatine modifiée avec des dérivés ammonium, la gélatine modifiée avec des groupes succinyle, la gélatine modifiée avec des groupes alcool vinylique, la gélatine modifiée avec des groupes vinylpyrrolidone, la gélatine hydrolysée, le poly(alcool vinylique) (PVA), la polyvinylpyrrolidone (PVP), le poly-(oxyde d'éthylène) (PEO), le polyacrylamide, le polyacrylate et leurs mélanges.

10. Milieu selon la revendication 9, dans lequel le polymère hydrosoluble comprend la gélatine, le poly(alcool vinylique) (PVA), la polyvinylpyrrolidone (PVP), le poly(oxyde d'éthylène) (PEO) ou leurs mélanges.

11. Milieu selon les revendications 1 à 10, dans lequel le polymère hydrosoluble comprend la gélatine avec une masse moléculaire moyenne comprise entre 1 kD et 200 kD, ou le poly(alcool vinylique) (PVA), la polyvinylpyrrolidone (PVP), le poly(oxyde d'éthylène) (PEO) ou des mélanges de polymères synthétiques ayant une masse moléculaire moyenne comprise entre 14 kD et 200 kD.

12. Milieu selon la revendication 11, dans lequel le polymère hydrosoluble comprend la gélatine avec une masse moléculaire moyenne comprise entre 1 kD et 50 kD, ou le poly(alcool vinylique) (PVA), la polyvinylpyrrolidone (PVP), le poly(oxyde d'éthylène) (PEO) ou des mélanges de polymères synthétiques ayant une masse moléculaire moyenne comprise entre 60 kD et 180 kD.

13. Milieu selon les revendications 1 à 12, dans lequel le point isoélectrique (IEP) dudit polymère hydrosoluble est dans la gamme de pH de 3,5 à 12.

14. Milieu selon les revendications 1 à 13, dans lequel le tensio-actif est choisi dans le groupe formé par les tensio-actifs anioniques, cationiques, non ioniques et amphotères.

15. Milieu selon la revendication 14, dans lequel le tensio-actif est choisi parmi les tensio-actifs anioniques contenant des alkylarylsulfonates, des esters de sulfate et des sulfonates aliphatiques, et parmi les tensio-actifs cationiques contenant des composés d'ammonium quaternaire.

16. Milieu selon les revendications 1 à 15, dans lequel la solution aqueuse contient en outre des additifs en une quantité inférieure à 45% en poids de la solution aqueuse.

17. Milieu selon la revendication 16, dans lequel la quantité d'additifs est inférieure à 35% en poids de la solution aqueuse.

18. Milieu selon la revendication 16 ou 17, dans lequel la quantité d'additifs est comprise entre 1% et 30% en poids de la solution aqueuse.

19. Milieu selon l'une quelconque des revendications 16 à 18, dans lequel lesdits additifs comprennent des particules colloïdales non poreuses choisies dans le groupe constitué par les particules siliceuses, l'oxyde d'aluminium et le carbonate de calcium, ou des particules poreuses dont la boéhmite, la pseudo-boéhmite, la silice précipitée, le gel de silice et la silice pyrogénée, et leurs mélanges.

20. Milieu selon la revendication 19, dans lequel la taille desdites particules colloïdales est comprise entre 5 et 700 nm.

21. Milieu selon la revendication 20, dans lequel la taille desdites particules colloïdales est comprise entre 5 et 100 nm.

22. Milieu selon la revendication 21, dans lequel la taille desdites particules colloïdales est comprise entre 5 et 70 nm.

23. Milieu selon les revendications 19 à 22, dans lequel lesdits additifs comprenant des particules poreuses ont une taille moyenne de particules comprise entre 100 et 2000 nanomètres.

24. Milieu selon la revendication 23, dans lequel la taille des pores desdites particules poreuses est comprise entre 1 et 500 nanomètres.

25. Milieu selon les revendications 1 à 24, dans lequel ledit film microporeux peut être obtenu par un procédé de fabrication comprenant les étapes consistant à mélanger une résine thermoplastique orientable avec au moins une charge enduite, à extruder ledit mélange à haute température pour former un film de celui-ci, à pré-étirer le film, à refroidir ledit film jusqu'à solidification du film et à étirer ledit film refroidi pour former un film microporeux.

26. Milieu selon les revendications 1 à 25, dans lequel ledit film microporeux comprend 30% à 90% en poids de charge.

27. Milieu selon les revendications 1 à 26, dans lequel ladite charge comprend le carbonate de calcium, le sulfate de baryum, la silice, le dioxyde de titane ou un mélange de ceux-ci.

28. Milieu selon les revendications 1 à 27, dans lequel ladite charge présente une taille moyenne de particules inférieure à 40 µm.

29. Milieu selon la revendication 28, dans lequel ladite charge présente une taille de particules moyenne de préférence comprise entre 0,5 et 10 µm.

30. Milieu selon les revendications 25 à 29, dans lequel la résine thermoplastique comprend le polyéthylène, le polypropylène, les copolymères d'éthylène et d'alpha-oléfines, les copolymères d'éthylène et d'acides acryliques, les copolymères d'éthylène et d'acides méthacryliques, les copolymères d'éthylène et d'acétate de vinyle, les copolymères de propylène et d'alpha-oléfines, le poly(chlorure de vinylidène), les copolymères de chlorure de vinylidène et d'acétate de vinyle, les copolymères de chlorure de vinylidène et de chlorure de vinyle, les copolymères d'éthylène et de propylène, les copolymères d'éthylène et de butène, le poly(acétate de vinyle), le polystyrène, le poly(acide omega-amino-undécanoïque), le poly(méthacrylate de méthyle), le poly(adipamide d'hexaméthylène) et/ou le poly-(epsilon-caprolactame).

31. Milieu selon la revendication 30, dans lequel la résine thermoplastique comprend le polyéthylène ; le polypropylène ; les copolymères d'éthylène et d'alpha-oléfines ; les copolymères éthylène/acétate de vinyle, les copolymères éthylène/acrylate de méthyle, les copolymères éthylène/acrylate d'éthyle, les copolymères éthylène/acide acrylique ; et les ionomères, et leurs mélanges.

32. Milieu selon les revendications 1 à 31, dans lequel ledit support est un papier de support photographique, un papier synthétique ou un substrat de film.

33. Milieu selon les revendications 1 à 32, dans lequel ledit support est stratifié sur une face avec une matrice polymère comprenant au moins une résine polyoléfinique.

34. Milieu selon les revendications 1 à 33, dans lequel ladite couche réceptrice d'encre comprend des particules absorbantes et un liant.

35. Milieu selon la revendication 34, dans lequel lesdites particules absorbantes dans la couche réceptrice d'encre sont la silice, la boéhmite, la pseudo-boéhmite ou une combinaison de celles-ci.

36. Milieu selon la revendication 34 ou 35, dans lequel ledit liant dans la couche réceptrice d'encre comprend les gélatines, le poly(alcool de vinyle), la polyvinylpyrrolidone, les dérivés de cellulose ou leurs mélanges.

37. Milieu selon les revendications 1 à 36, comprenant en outre une couche protectrice perméable à l'encre par-dessus ladite couche réceptrice d'encre.

38. Milieu selon la revendication 37, dans lequel ladite couche protectrice comprend l'hydroxypropylméthylcellulose, le poly(alcool de vinyle) ou une solution de gélatine.

39. Procédé de préparation d'un milieu d'enregistrement pour jet d'encre comprenant les étapes consistant à :
a. pré-traiter un film microporeux hydrofuge avec une solution aqueuse comprenant au moins un polymère hydrosoluble et un tensio-actif, ledit film microporeux étant un film thermoplastique orienté comprenant des charges et comportant des canaux d'interconnexion entre les pores, avec un volume de vide compris entre 30% et 90% en volume de l'ensemble du film microporeux ;
b. faire adhérer ledit film sur un milieu ;
c. déposer une couche réceptrice d'encre sur ledit film ; puis éventuellement
d. déposer une couche protectrice par-dessus ladite couche réceptrice d'encre ; dans lequel l'étape a est réalisée avant l'étape c.

40. Procédé selon la revendication 39, dans lequel l'étape a est réalisée avant l'étape b.

41. Procédé de formation d'une image nette et permanente par jet d'encre comprenant les étapes consistant à :
- fournir un milieu d'enregistrement pour jet d'encre selon l'une quelconque des revendications 1 à 38
- introduire de l'encre pour jet d'encre en contact avec le milieu selon le motif d'une image souhaitée.

42. Film microporeux hygroscopique et hydrophile, pouvant être obtenu en imprégnant un film hydrofuge comprenant un thermoplastique orienté et au moins une charge, lequel film est perméable à l'air et à la vapeur d'eau et présente un volume de vides compris entre 30% et 90% en volume de l'ensemble du film, avec une solution aqueuse comprenant au moins un polymère hydrosoluble et un tensio-actif.
